

## UNITED STATES PATENT OFFICE

2,469,611

## PATTERN MATERIALS

Kenneth E. Rose, Columbus, Ohio, assignor, by  
mesne assignments, to United Aircraft Cor-  
poration, East Hartford, Conn., a corporation  
of Delaware

No Drawing. Application March 23, 1946,  
Serial No. 656,777

3 Claims. (Cl. 22—164)

1

This invention relates to pattern materials and particularly to pattern materials especially suitable for precision investment-casting processes.

In the precision investment-casting process, a pattern is cast in a pattern mold and an investment material is cast around the pattern. The investment mold thus formed is then heated and the pattern is removed, as by melting, burning, volatilization, or chemical decomposition, leaving the desired cavity in the mold. It has been the customary practice to make the patterns from wax or wax-like materials, since they may be readily removed at relatively low temperatures. The principal use of precision investment-casting was, in its early stages, in the dental industry where the pattern material had to melt at temperatures only slightly above body temperature and solidify at body temperature due to its use in the mouth of the patients. Subsequent advances in the precision investment-casting art have widened the use of this type of casting, and it is now used in many other fields, for example, in casting blades for turbo-superchargers for aircraft engines.

Although there is little information as to particular pattern materials which are especially suitable for precision investment-casting, the requirements of such materials are critical and well known in the art. In the first place, it is essential that the pattern material be capable of reproducing with great accuracy the contours of the pattern mold. In order to achieve such reproducibility, it is desirable to have low thermal expansion, low viscosity of pattern material when molten, fine grain structure, and a pattern material of crystalline nature. Secondly, it is desirable that the pattern material be characterized by sufficient strength and resilience to prevent cracking of the pattern when cast in a mold offering resistance to shrinkage. Furthermore, the pattern material should be hard and have very little, if any, cold flow in order that the pattern will not materially alter in contour from the time it is cast until the time the investment is cast around it. Finally, it is highly important that the pattern material be characterized by uniform shrinkage regardless of the temperature at which it is poured. The present casting waxes and other pattern materials have failed to fulfill these requirements and, as a result, the employment of precision investment-casting processes has been generally restricted to small castings, thus eliminating the production of many of the more important products which might be precision made.

It is, therefore, an object of this invention to provide a pattern material capable of highly accurate reproduction of the contours of the pattern mold.

Another object of this invention is to provide a pattern material that may be readily cast in

2

molds of intricate design which offer resistance to the shrinkage of the pattern material.

It is a further object of this invention to provide pattern materials characterized by considerable cold flow stability and hardness so as to prevent distortion between the time of molding and the time that the investment is cast about the pattern.

Still another object of this invention is to provide a pattern material characterized by uniform shrinkage regardless of the temperature at which the pattern material is poured.

Yet another object of this invention is to provide a pattern material satisfactory for casting large objects with the precision investment-casting method.

Other objects and advantages of the present invention will become apparent from the following detailed description thereof.

The present invention comprises, in general, a pattern material consisting essentially of a mixture of hydrogenated castor oil and chlorinated naphthalene in certain proportions. Neither of these two materials by itself is satisfactory as a pattern material; the hydrogenated castor oil has very poor castability because of its brittleness and the chlorinated naphthalene has such a large grain structure that it does not reproduce the contours of the pattern mold with sufficient accuracy. When mixed together, these two compounds do not generally produce a satisfactory pattern material, but it has been discovered that those mixtures containing between about 60 and about 80% chlorinated naphthalene and between about 40 and about 20% hydrogenated castor oil produce a wax remarkably suited to use as a pattern material in precision-casting processes.

It is readily apparent that the first and foremost requirement of a pattern material is a high degree of reproducibility, since without that the pattern is of no value whatsoever. It should be kept in mind that these patterns herein referred to are employed in precision investment-casting processes wherein the accuracy of reproduction is generally the sole justification for the greatly added cost of casting metal in this manner. Since mixtures of hydrogenated castor oil and chlorinated naphthalene containing from about 60 to about 80% chlorinated naphthalene have very low viscosity when molten, they readily reproduce the contours of the mold. The principal limitation on the reproductive qualities of such mixtures is the growth of grain size which becomes clearly noticeable in compositions containing much more than 80% chlorinated naphthalene.

Not only are such mixtures of chlorinated naphthalene and hydrogenated castor oil capable of reproducing the contours of the pattern mold, but they are exceptionally castable, that

is, they are characterized by sufficiently low thermal expansion, high strength, and resilience to prevent cracking of the pattern from cooling in intricate molds which present considerable resistance to shrinkage. In the following Table 1, the per cent of volumetric thermal expansion which occurs upon heating the pattern material from 20° C. to its melting point is shown for various mixtures of hydrogenated castor oil and chlorinated naphthalene (49% chlorine).

Table 1

| Hydrogenated Castor Oil-Chlorinated Naphthalene Mixture | Volumetric Thermal Expansion, percent |
|---------------------------------------------------------|---------------------------------------|
| 30% chlorinated naphthalene                             | 8.0                                   |
| 40% chlorinated naphthalene                             | 7.8                                   |
| 50% chlorinated naphthalene                             | 8.6                                   |
| 60% chlorinated naphthalene                             | 6.7                                   |
| 75% chlorinated naphthalene                             | 5.4                                   |
| 80% chlorinated naphthalene                             | 5.3                                   |
| 90% chlorinated naphthalene                             | 3.5                                   |

The fact that the peak of thermal expansion lies at about 50% chlorinated naphthalene accounts, at least in part, for the rapid decrease in castability of compositions containing less than 60% chlorinated naphthalene. This lower limit is further established by the embrittling action encountered in compositions containing in excess of 40% hydrogenated castor oil. Statistical affirmation of this observed result is found in the following Tables 2 and 3, which show, respectively, the relative transverse strength and the deflection of different mixtures of hydrogenated castor oil and chlorinated naphthalene (49% chlorine).

Table 2

| Hydrogenated Castor Oil-Chlorinated Naphthalene Mixture | Transverse Strength, Pounds |
|---------------------------------------------------------|-----------------------------|
| 20% chlorinated naphthalene                             | 4.5                         |
| 30% chlorinated naphthalene                             | 5.2                         |
| 50% chlorinated naphthalene                             | 6.5                         |
| 60% chlorinated naphthalene                             | 8.0                         |
| 80% chlorinated naphthalene                             | 8.8                         |
| 90% chlorinated naphthalene                             | 8.0                         |

The transverse strength of a given pattern material is determined by suspending a weight at the middle of a bar of the pattern material having a cross-section of  $\frac{1}{2} \times \frac{3}{8}$  inch and a span of 3 inches. The deflection is measured directly below the point of application of the load, and represents the ability of the pattern material to bend before breakage occurs.

Table 3

| Hydrogenated Castor Oil-Chlorinated Naphthalene Mixture | Deflection in .001 inch |
|---------------------------------------------------------|-------------------------|
| 20% chlorinated naphthalene                             | 14                      |
| 30% chlorinated naphthalene                             | 19                      |
| 50% chlorinated naphthalene                             | 27                      |
| 60% chlorinated naphthalene                             | 27                      |
| 80% chlorinated naphthalene                             | 51                      |
| 90% chlorinated naphthalene                             | 46                      |

It is apparent from the above Tables 2 and 3 that both the transverse strength and the resilience, or deflection, of the hydrogenated castor oil-chlorinated naphthalene mixtures decrease markedly below 60% chlorinated naphthalene. As a result, the lower limit of 60% chlorinated naphthalene not only marks the point below which successful casting of these waxes becomes

extremely difficult, but also indicates a limit below which the embrittling action of the hydrogenated castor oil makes handling of the molded patterns hazardous. As will be hereinafter pointed out, 5 slightly lower percentages of naphthalene chloride may be employed when the naphthalene chloride employed is of a degree of chlorination materially greater than 49% chlorine.

Mixtures of hydrogenated castor oil and chlorinated naphthalene containing as high as 90% of the latter have suitable properties for pattern materials, but the use of such compositions containing in excess of 80% chlorinated naphthalene is impractical. The present commercial practice 10 is to employ chilled molds for forming patterns in order to reduce the time required for cooling the pattern material and, consequently, reducing the molding period. Due to the rise in melting point of mixtures containing more than 80% 15 chlorinated naphthalene, the temperature differential between such mixtures and the chilled molds results in cracked patterns. Patterns may be cast satisfactorily, however, using compositions containing up to 90% chlorinated naphthalene if the molds are warm, and even where the molds are cold if the pattern is quite large so that the chilling effect is minimized.

The hydrogenated castor oil used is principally 20 a 12-hydroxy stearin (glyceryl trihydroxy stearate). The chlorinated naphthalene employed can vary in degree of chlorination between naphthalene trichloride and naphthalene hexachloride. The chlorination of naphthalene results in a 25 product comprising a mixture of different chlorides, so that it is more practical to define this product according to chlorine content, density, melting point, etc. Thus, chlorinated naphthalene having a chlorine content of about 49% and having a melting point of about 80° C. has been 30 found to be very satisfactory, and another chlorinated naphthalene having a chlorine content as high as 61% has been found to be even better for certain purposes.

The proportions in which the various ingredients are present depends upon the degree of chlorination of the naphthalene chloride. Thus, for 35 chlorinated naphthalenes having a chlorine content of about 49%, mixtures of hydrogenated castor oil and chlorinated naphthalene in which the chlorinated naphthalene is present to the extent of from about 60 to about 80% have proven 40 very satisfactory as pattern materials. Where the naphthalene has been chlorinated to a higher degree, such as that containing about 61% chlorine, the amounts of chlorinated naphthalene 45 may be reduced to as low as 50% and still provide satisfactory pattern materials. A mixture which has been found to be especially advantageous 50 when using any of the chlorinated naphthalenes containing chlorine within the range of about 49% to about 61%, comprises about 25% hydrogenated castor oil and about 75% chlorinated naphthalene.

The chlorinated naphthalene being actually a 55 mixture of several compounds, does not form a true binary system with the hydrogenated castor oil so as to permit accurate predictions of melting points, freezing points, and other physical properties, from the properties of the previously known mixtures of these two compounds. Consequently, the discovery that compositions of hydrogenated castor oil and chlorinated naphthalene containing from about 60 to about 80% chlorinated naphthalene were particularly adapted

for use as pattern materials was an unpredictable development.

In summary, the present invention lies in the discovery that a relatively narrow range of the mixture of hydrogenated castor oil and chlorinated naphthalene may be employed satisfactorily as pattern materials, but mixtures falling within this range, indicated for most purposes by those mixtures containing between 60 to 80% chlorinated naphthalene, have excellent properties which especially suit them for production of patterns. Such materials have a very high degree of accuracy of reproduction and may be readily cast in the most intricate molds. Upon removal from the pattern mold, patterns made of the mixtures comprising the present invention will retain their dimensions within very close tolerances over long periods of time. The extremely low viscosity of the molten hydrogenated castor oil-chlorinated naphthalene mixtures makes it possible to gravity cast as well as to injection mold the patterns. This latter feature is of especial importance in that a considerable saving is realized by elimination of highly expensive mechanisms required for molding under pressure. Another characteristic of especial importance of the present pattern materials is the uniform shrinkage obtained regardless of the pouring temperature. High dimensional accuracy of the part to be molded by precision casting is generally required, so that it is necessary to allow for even slight shrinkage of the pattern upon cooling. This can be done satisfactorily on a commercial basis only where the shrinkage is uniform regardless of slight variations, or even large variations, in the pouring temperature. Still another factor of considerable commercial importance is the reduced cost of the present pattern material when compared with pattern materials heretofore in general use. Still another feature is the excellent

machinability of this pattern material which permits drilling, threading, or turning to provide features that might be difficult to incorporate in a pattern mold.

A number of variations of the present invention will become apparent to those skilled in the art upon reading this disclosure, and such variations or modifications as fall within the appended claims constitute a part of the present invention.

What is claimed is:

1. A pattern material consisting essentially of a mixture of hydrogenated castor oil and chlorinated naphthalene in which the latter compound is present in the mixture to the extent of from about 60% to about 90% and has a chlorine content of about 49% to about 60%.

2. A pattern material consisting essentially of a mixture of hydrogenated castor oil and chlorinated naphthalene, said mixture containing about 60% to about 80% of chlorinated naphthalene which has a chlorine content of about 49% to about 61%.

3. A pattern material consisting essentially of about 25% hydrogenated castor oil and about 75% chlorinated naphthalene having a chlorine content of from 49% to about 61%.

KENNETH E. ROSE.

#### REFERENCES CITED

30 The following references are of record in the file of this patent:

#### UNITED STATES PATENTS

| Number    | Name              | Date          |
|-----------|-------------------|---------------|
| 2,133,300 | Linebarger et al. | Oct. 18, 1938 |
| 2,266,813 | Ruben             | Dec. 23, 1941 |

#### OTHER REFERENCES

The Foundry, page 184, "Wax Compositions,"  
40 April 1944.